

106. COMPOSITIONS,  
COATING OR PLASTIC

CROSS REFERENCE

84 -M

Examiner

Feb. 16, 1932.

J. W. ANDREWS ET AL

1,845,113

MAGNETIC MATERIAL AND MAGNET CORE

Filed Dec. 31, 1927

Fig. 1.



Fig. 2.



Inventors  
John W. Andrews  
Randall Gillis  
by H. Sattler, Att'y.

106-84M

Patented Feb. 16, 1932

1,845,113

XR

# UNITED STATES PATENT OFFICE

JOHN WENDELL ANDREWS, OF CHICAGO, AND RANDALL GILLIS, OF BERWYN, ILLINOIS,  
ASSIGNORS TO WESTERN ELECTRIC COMPANY, INCORPORATED, OF NEW YORK, N. Y.,  
A CORPORATION OF NEW YORK

## MAGNETIC MATERIAL AND MAGNET CORE

Application filed December 31, 1927. Serial No. 244,020.

This invention relates to magnetic materials and magnet cores, and especially to magnetic cores for loading coils for use in telephone circuits.

The principal object of the invention is the production of magnetic elements having stable magnetic properties under varying magnetic conditions.

Another object of the invention is the production of magnetic elements having low core losses and a relatively high permeability to enable a given inductance to be obtained from a minimum amount of material, and possessing to a high degree those electrical and magnetic characteristics which make it highly desirable in electrical signalling apparatus, particularly in loading coils for telephone circuits.

In accordance with one embodiment, the present invention contemplates the construction of magnetic cores of an alloy including nickel and iron in finely divided form, heat treated to have a higher inherent magnetic permeability and lower inherent hysteresis loss than iron, and combined with a suitable insulating material. More specifically, the invention contemplates the formation of magnetic cores of a nickel-iron alloy in finely divided form in which the proportions of its constituents are such that the resulting alloy has the maximum magnetic stability. The metal particles are treated with a refractory insulating material whereby the alloy particles are individually insulated after which they are compressed into cores of the desired shape and size. The cores are heat treated at the optimum temperature for the particular alloy of which they are constructed to give the cores the desired mechanical, electrical and magnetic characteristics.

It is believed that the invention will be clearly understood from the following detailed description of one embodiment thereof and the accompanying drawings, in which

Fig. 1 is a perspective view of a section of a loading coil core made in accordance with the present invention, and

Fig. 2 shows a plurality of these sections assembled to form a completed core.

It will be understood, however, that this is

merely illustrative and the invention is not limited to the production of this form of core, but is adapted to the production of cores for magnetic articles of many forms.

In carrying out the present invention the magnetic material is prepared in the following manner. The magnetic material employed is prepared from a nickel-iron alloy commonly referred to as "permalloy", which is treated in a manner more fully described in the copending application of H. M. E. Heinicke, Serial No. 229,801, filed October 29, 1927, to reduce the alloy to a finely divided form. Experience has proven that where low eddy current losses are desired it is essential that the particles be of a small size and preferably of such size that all of the particles will readily pass through what is generally known as a 120 mesh screen and a large percentage pass through a 200 mesh screen. According to one embodiment of the invention, the alloy is prepared by melting approximately 80 parts of nickel and 20 parts of iron in an oxidizing atmosphere and pouring the resulting alloy into a mold. When prepared according to the foregoing process, the resulting alloy will be exceedingly brittle and it is therefore particularly adapted to be reduced to a finely divided or dust form from which cores may be molded.

The brittle ingots obtained from the above described process are successively passed through progressively reducing hot rolls which decrease the cross sectional dimensions of the piece of material and the final roll is effected at approximately the temperature at which the alloy ceases to be malleable, after which the rolled material is quenched to a temperature below that at which it loses its malleability. By the hot rolling and quenching process the size of the crystalline structure is materially reduced, which is very desirable because disintegration of the material takes place mainly at the crystal boundaries, and consequently the smaller the size of the crystals the finer the dust which can be produced from the finished product. The rolled and quenched material is broken into short pieces and the pieces are crushed in a jaw crusher, hammer mill, or any other suit-

able type of apparatus, after which the crushed material is reduced to a fine dust in a ball mill or any other suitable pulverizing device. The dust is sieved through a 120 mesh sieve and any residue is remelted and again carried through the above described operations to reduce the material to a finely divided form.

The finely divided magnetic material obtained by the above described operations is particularly adapted to be formed into rings or cores for loading coils by individually insulating the particles with a refractory insulating material and compressing the insulated particles. The particles may be insulated in accordance with the method described more fully in our copending application, Serial No. 102,729, filed April 17, 1926, in which method the finely divided particles of the nickel-iron alloy are annealed in a closed container at a temperature of approximately 925° C., after which the resulting cake of annealed alloy is again reduced to a finely divided form. The annealed particles are then individually insulated with a refractory insulator comprising approximately:

5 1/2 parts of chromic acid  
5 parts of talc  
4 1/2 parts of water glass composed of 50% total solids and containing approximately 1.58 parts of  $\text{SiO}_2$  to 1 part of  $\text{Na}_2\text{O}$ .

The insulated dust particles are then in a form suitable for pressing into cores or rings which are preferably formed with a pressure of approximately 200,000 pounds per square inch. A high pressure is used in forming the rings in order to increase their density, since it has been found that the permeability of the rings increases with increased density. Following this step, the cores are transferred without unduly exposing them to the air into an annealing furnace in which they are annealed at the optimum annealing temperature of approximately 500° C. and cooled. If necessary, the cores may be boiled in water to remove soluble substances and to render the cores chemically stable, and dried at a temperature of approximately 100° C.

A plurality of rings thus formed are then stacked coaxially to form a core on which the usual toroidal winding is applied, the number of such rings used depending upon the existing electrical characteristics of the telephone circuit with which the loading coils are to be associated.

Although the alloy has been described as being composed of approximately 80% nickel and the remainder principally iron, it is to be understood that the proportions of the ingredients may be varied without departing from the spirit and scope of the invention. For example, nickel-iron alloy having substantially stable magnetic properties may be produced by employing from

79% to 84% nickel. Furthermore, other refractory insulating materials than those described in the specific example given hereinbefore may be employed with satisfactory results. For instance, the articles may be insulated with a material consisting of kaolin and boric acid, or a mixture of sodium aluminate and kaolin. Or, the particles may be treated chemically to produce a coating composed of the oxides of the constituents of the alloy upon the particles. In fact, any insulating material which will serve to individually insulate the finely divided particles and which will withstand the effects of the annealing treatment to which the compressed rings are subjected may be employed with satisfactory results.

By the term "magnetic stability" which is employed hereinbefore in the specification and hereinafter in the annexed claims, is meant that the permeability of the material and consequently the inductance of a coil employing such material is substantially unaffected by instantaneous direct current magnetizations. The magnetic stability of the alloy may be computed from the difference in the inductance of a coil before and after being subjected to an instantaneous direct current magnetization, and may be expressed by the following formula:

$$S = 100 - \frac{100\Delta L}{L}$$

in which S is the percent magnetic stability,  $\Delta L$  is the change in inductance, and L is the original inductance before the instantaneous direct current magnetization. For an alloy containing approximately 80% nickel and the remainder principally iron, the value

$$\frac{100\Delta L}{L},$$

which represents the percent change in inductance produced by the instantaneous direct current magnetization, falls within the limits of  $\pm .5\%$  and consequently the magnetic stability, represented by the letter S, for an alloy containing approximately 80% nickel is 99.5% to 100.5%.

By using an alloy of the proportions stated in the preceding paragraphs and by following the foregoing method of insulating the individual alloy particles and compressing the particles into cores or rings, magnetic structures are produced which have an extremely high magnetic stability and permeability from the minimum amount of material. By the use of such cores or rings, inductance units having a high magnetic stability, having the same permeability with equal or less hysteresis and eddy current losses as cores constructed according to previously known methods, but with much less core volume and much less coil volume, are available.

What is claimed is:

1. A magnetic core of high magnetic stability composed of finely divided individually insulated particles of an alloy of approximately 80% nickel and 20% iron annealed at a temperature of approximately 925° C. formed into shape under a pressure of approximately 200,000 pounds per square inch and annealed as a whole at a temperature of approximately 500° C.
2. The process of manufacturing magnetic cores of high magnetic stability which consists in reducing an alloy of approximately 80% nickel and 20% iron to dust, annealing the dust at a temperature of approximately 925° C., reducing the annealed cake to dust again, coating the particles of dust with a refractory insulating material, pressing the insulated dust into form under a pressure of approximately 200,000 pounds per square inch, and annealing the formed cores at a temperature of approximately 500° C.
3. A magnetic core of high magnetic stability comprising finely divided individually insulated particles of an alloy comprising from 79% to 84% nickel and the remainder principally iron annealed at a temperature of the order of 925° C. formed into shape under a pressure of the order of 200,000 pounds per square inch and annealed as a whole to produce a high magnetic stability.

In witness whereof, we hereunto subscribe our names this 24th day of December, A. D. 35 1927.

JOHN WENDELL ANDREWS.  
RANDALL GILLIS.

40

45

50

55

60

65